

Patented July 29, 1924.

1,502,705

# UNITED STATES PATENT OFFICE.

WILLIAM P. WITHEROW, OF PITTSBURGH, PENNSYLVANIA, ASSIGNOR TO WITHEROW STEEL COMPANY, OF NEVILLE ISLAND, PENNSYLVANIA, A CORPORATION OF PENNSYLVANIA.

## METHOD OF DIE ROLLING.

No Drawing.

Application filed September 9, 1922. Serial No. 587,080.

To all whom it may concern:

Be it known that I, WILLIAM P. WITHEROW, a citizen of the United States, residing at Pittsburgh, in the county of Allegheny and State of Pennsylvania, have invented a new and useful Improvement in Methods of Die Rolling, of which the following is a full, clear, and exact description.

The present invention relates broadly to metal working, and more particularly to die rolling methods in which accuracy in the dimensions of the finished product is important.

At the present time, considerable difficulty is encountered in the die rolling art in the production of finished articles or blanks having accurate and uniform dimensions. Many attempts have been made to produce blanks for certain purposes, but due to the variations in the dimensions many of these attempts have been abandoned.

In the metal rolling art, other than die-rolling, it is customary to produce variations in the dimensions of rolled articles by changing the temperature of the ingot being rolled, the temperature being increased when it is desired to increase the dimensions of the article. By increasing the temperature it is not unlikely that increased dimensions are insured due to the fact that the ease of flow of the metal under the action of the rolls is increased.

By continued investigation and repeated experiments in the die rolling art in which the reductions of the leader throughout its length may vary to produce the blanks, I have found that in order to increase the length of a die rolled blank the reverse effect occurs, so that it is necessary to decrease the temperature of the billet or leader being rolled, while to decrease the length of the rolled blank it is essential to increase the temperature of the billet or leader. I have also found that the variations produced in the lengths of blanks by reason of changes in the temperature of the billet or leader, as referred to, vary in accordance with the reduction which is being effected on the billet or leader by the die rolls. In other words, as the per cent of reduction increases, an increase in temperature will produce a shorter blank than will be produced at the same temperature if the per cent of reduction is decreased.

In accordance with the present invention, the temperature of the entering material is decreased to produce longer blanks and increased to produce shorter blanks, the variations in the temperature being figured in accordance with the percentage of reduction being effected by the die rolls. It is believed that these results are accomplished for the reason that as the temperature of the metal is increased the slippage between the rolls and the metal is increased, thereby resulting in a shorter product; while if the temperature is decreased the effective grip on the metal is increased, thereby subjecting the same to an increased rolling action which effects a greater flow of metal and consequently a longer blank. These results may, however, be due to other causes.

In other words, the process is carried out by noting the temperature at which what might be called test leaders, are passed through the rolls, and such die-rolled blanks are then measured and the necessary corrections for length of the successive die-rolled blanks are then made by passing the leaders to the rolls at a lower temperature, than the above mentioned leaders, if longer blanks are desired or at a higher temperature if shorter blanks are desired.

The advantages of the present invention arise from the method of insuring uniform results in an expeditious manner by merely varying the temperature at which the metal is fed to the die rolls to control the length of the blank.

I claim:

1. The method of die-rolling blanks of predetermined length from leaders, comprising the step of passing a heated leader at a given temperature through a die-roll pass, and then die-rolling similar blanks from successive leaders by delivering such leaders to the die-rolls at a reduced temperature if longer blanks are desired.

2. The method of die-rolling blanks of predetermined length from leaders, comprising the step of passing a heated leader at a given temperature through a die-roll pass, and then die-rolling similar blanks from successive leaders by delivering such leaders at a higher temperature if shorter blanks are desired.

3. The method of die-rolling blanks of predetermined length from leaders, comprising the step of passing a heated leader

at a given temperature through a die-roll pass, and then die-rolling similar blanks from successive leaders by delivering such leaders to the die-rolls at a reduced temperature if longer blanks are desired, such reduction in temperature being in accordance with the percentage of reduction of the blank.

4. The method of die-rolling blanks of 5 predetermined length from leaders, comprising the step of passing a heated leader

at a given temperature through a die-roll pass, and then die-rolling similar blanks from successive leaders by delivering such leaders at a higher temperature if shorter 15 blanks are desired, such increase in temperature being in accordance with the percentage of reduction of the blank.

In testimony whereof I have hereunto set my hand.

WILLIAM P. WITHEROW.